

Oct. 4, 1927.

1,644,389

M. L. MARTUS ET AL

PRIMARY CELL AND METHOD OF MAKING THE SAME

Filed Jan. 3, 1927



Patented Oct. 4, 1927.

1,644,389

# UNITED STATES PATENT OFFICE.

MARTIN L. MARTUS, OF WOODBURY, AND EDMUND H. BECKER, OF WATERBURY,  
CONNECTICUT.

## PRIMARY CELL AND METHOD OF MAKING THE SAME.

Application filed January 3, 1927. Serial No. 158,694.

This invention relates to primary cells and methods of making the same; and it comprises a new primary cell of the Lalande type having an alkaline electrolyte, a zinc pole 5 and a copper oxid pole, the latter carrying a facing of reduced copper and being protected by a layer of preshrunk zincated paper or fabric; and it also comprises a method of making such cells wherein paper or fabric 10 is preshrunk and impregnated with zinc by a treatment with sodium zincate, the preshrunk fabric being further treated with a solution of sodium and/or potassium silicate, dusted with a powdered metal electropositive to copper, such as metallic zinc, and wrapped around a copper oxid pole with the face carrying the zinc next the oxid, the whole then being assembled with the other 15 elements of a Lalande cell; all as more fully 20 hereinafter set forth and as claimed.

For closed circuit work, the type of cell employing copper oxid against zinc in a caustic soda electrolyte is practically the only one used. It is not well adapted for 25 open-circuit work and shelf loss is apt to be considerable; both facts being largely due to the solubility of copper oxid in solutions of caustic soda or of caustic potash. While this solubility is very small, it is nevertheless 30 sufficient to allow migration of copper by a diffusion and convection to the zinc in time. Copper reaching the zinc produces local 35 action. On closed circuit the caustic soda solution is kept stripped of copper and this action does not occur. Solubility of copper in the caustic soda solution is aided by many 40 organic impurities but, on the other hand, copper can be withdrawn from the solution by cellulose and some other substances. Alkali cellulose, which is a condition in 45 which cellulose must occur in such a cell, is fairly active in withdrawing copper from the electrolyte. Cotton cloth, paper, etc., are often used in this type of cell for structural 50 reasons and in so doing, they have the additional utility of withdrawing copper from the electrolyte. We have found, however, that paper and cloth treated with a sodium zincate solution possess this absorbing 55 power for copper in a considerably increased degree and in our copending application, Serial No. 157765, we have described and claimed various cells utilizing this property. In the present invention, we also utilize paper or cloth so treated.

In the Lalande type of cell, sometimes the copper oxid is employed as a granular mass supported in suitable ways and sometimes it is formed into a solid body by appropriate treatments. In either event, it is customary 60 to metallize the outer surfaces by some sort of a reducing treatment; that is, the copper oxid is superficially converted into copper before assembling the cell. This is an item of some expense in the manufacture of these 65 cells.

In the present invention, we utilize the copper stopping properties of zincated cellulose, using a sheet of this material for surrounding the copper oxid pole. And before 70 assembling the sheet with the copper oxid, the sheet is surfaced with fine zinc dust. On assemblage of the zinc-strewn zincated paper with the copper oxid pole and wetting, the zinc superficially reduces the copper oxid 75 and is itself converted into sodium zincate which passes into the paper. The paper is locally treated with a solution of sodium zincate of high concentration. In specific 80 embodiments of the present invention, we take cheesecloth or paper and immerse it in a strong solution of zinc oxide in caustic soda or potash. Such a solution may be made directly by dissolving zinc or zinc oxide in caustic soda; but it is more economical to 85 employ exhausted battery solutions. On complete exhaustion Lalande type cells, having the usual strength of caustic soda electrolyte, give sodium zincate solutions of about 90 40° Baume. These are suitable for our purpose. On immersion in the zincate solution at the ordinary temperature, that is, a temperature of, say, 60° to 70° F., the paper 95 swells, and shortens and shrinks laterally. The total shrinkage may amount to a loss of 40 to 50 per cent of the square area. The paper takes up and holds zinc oxide. Swelling and adsorption are complete in a short time. In practicing our invention, the shrunk paper is withdrawn, slightly dried 100 and dipped in a solution of potassium or sodium silicate, this serving as an adhesive. The solution may be merely painted over one surface. On this painted surface is next dusted fine zinc powder. Aluminum 105 powder may be used. With aluminum powder, sodium aluminate is formed in the cell and reacts with the sodium silicate to form a layer of artificial zeolite, which is useful in removing copper from solution 110

(Martus & Becker Patent No. 1,581,851). A mixture of powdered zinc and aluminum may be used. Zinc and aluminum are both metals electropositive to copper. The paper 5 is next used as a wrapping for the copper oxide pole, being placed with the zinc or aluminum coated side next the oxid. Where the copper oxide is used as an outside annulus, the treated paper is placed on the inside 10 of the annulus. Where the copper oxide pole is central and cylindrical, the specially treated paper is wrapped around it with the zinc or aluminum surface inside.

The formation of sodium zincate in assembling the cell may be relied upon for impregnating the paper with zinc; but we ordinarily find it much better to preshrink the paper with zincate. As noted, shrinkage is considerable. Instead of using paper, 15 cheesecloth can be used.

In the accompanying illustration we have shown, more or less diagrammatically, an embodiment of the described invention. In this showing,

20 Figure 1 represents a cross section of an assemblage of cell elements;

25 Figure 2 represents a partial view in section taken along the line 2—2 of Figure 1, only half of the section being shown; and

30 Figure 3 shows in perspective paper separating means provided with a surfacing layer of zinc dust.

35 Referring more particularly to Figure 1, from the fragmentarily shown cover or top 1 of the cell jar container, depends a yoke 2 serving as a conductor and as a supporting means for the cell elements. Yoke 2 is carried by a bolt 3 passing through the top 1 and provided with nut 4, washers 5, and wing nut 6. Rods 7 pass through insulating carrier plate 8 and are bent upward at their lower ends as shown at 9 for the purpose of holding the cell assembly on the yoke 2 and for the purpose of supporting 40 the body of copper oxid 10, the treated paper 45 separators 11 and the perforated plates 12. An anode, in the form of a cylindrical zinc plate 13, is attached to the plate 8 by bolts 15 and wing nuts 14. A second annular 50 zinc anode 16 surrounds the cathode and is likewise held by bolts 15 by means of lugs 17. A terminal wire 18 is connected to bolt 15 and passes out through a hole in the cover of the cell container 1, as shown. 55 The annular cathodic element of copper oxid 10 is disposed between the two anodes 13 and 16. Annular paper sleeves 11 are placed inside and outside of the annular copper oxid cathode and around the paper sleeves there 60 are perforated metallic screens 12. In Figure 2 is shown the radial relationship of these elements. In Figure 3 the paper sleeve 11 is shown provided with a coating of zinc dust 11a.

In manufacturing the cells for use, the 65 cell is assembled as shown in Figure 1, with the paper sleeves 11 in place having their zinc coated surfaces adjacent the copper oxid cathode. The inner sleeve has its exterior face surfaced with zinc dust while the outer sleeve has its interior face surfaced with zinc dust. The cells are shipped and stored in a dry condition. Upon addition of the electrolyte to the cell, this electrolyte consisting of about a 20 per cent solution of caustic soda in water, the presence of the zinc next to the copper oxid surface causes a superficial reduction of the copper oxid cathode surfaces. In this way, the usual manufacturing operation of superficially 70 reducing the copper oxid is dispensed with and considerable time and expense in the manufacture of the cells are done away with.

What we claim is:—

1. In the process of manufacturing primary cells of the zinc-copper oxid type, the steps which comprise impregnating a paper sleeve with sodium zincate solution, superficially coating the so-treated paper with a solution of alkali silicate, sprinkling a thin layer of zinc dust on the paper while it is still wet with silicate solution, and thereafter placing said paper in a copper oxid-zinc cell with the metallized surface of said paper in contact with the copper oxid. 90

2. A new material for use in copper oxid-zinc cells comprising paper impregnated with sodium zincate solution and having a layer of zinc dust on one of said surfaces. 95

3. A primary cell comprising inner and outer zinc anodes, a body of copper oxid disposed between said anodes, sheets of paper disposed between the copper oxid and the zinc anodes, said paper carrying zinc dust on its surface, and said metallized surface being in contact with the copper oxid. 100

4. In a cell of the Lalande type, a layer of paper impregnated with sodium zincate solution and having a layer of metal dust on one surface of said paper. 105

5. In a cell of the Lalande type, a layer of paper impregnated with sodium zincate solution and having a layer of metal dust on one surface of said paper, said metal being electropositive to copper. 110

6. In a cell of the Lalande type, a layer of paper impregnated with sodium zincate solution and having a layer of zinc dust on one surface of said paper. 115

7. In a cell of the Lalande type, a layer of paper impregnated with sodium zincate solution and having a layer of zinc and aluminum dust on one surface of said paper. 120

In witness whereof we have hereunto signed our names at Waterbury, Connecticut, 125 this 31st day of December, 1926.

MARTIN L. MARTUS.  
EDMUND H. BECKER.